

## UNITED STATES PATENT OFFICE

WILLIAM ARTHUR WILLIAMS, OF EDINBURGH, SCOTLAND

## ELECTRODEPOSITION OF RUBBER

No Drawing. Application filed May 12, 1927, Serial No. 190,964, and in Great Britain February 7, 1927.

This invention relates to the electro-deposition of rubber or homologous substances from a vulcanized or unvulcanized preserved or alkaline latex.

5 A feature of the present invention is the elimination of any external source of electric current in the excitation of the electrolytic action, and to this end an electrolyte is selected which, when added to the 10 latex and used in conjunction with suitably selected electrodes directly connected together conductively outside the electrolyte, will act as a self-excitant, setting up an electromotive force sufficient to cause deposition 15 of rubber or homologous substances upon the anode element of the circuit, but insufficient to cause a decomposition which would produce gas bubbles at the anode.

In the collection of latex on the rubber 20 plantations for export in the latex form, it is usual to add an alkali such as ammonia for the purpose of preventing premature coagulation.

For the purpose of my process, it is desirable to reduce this alkalinity in the latex to 25 a minimum, and this is effected by the addition of an electrolyte which not only reduces the alkalinity to the necessary point, but also sets up with the electrodes a resulting chemical 30 action and electro-motive force in the circuit, which causes deposition of the rubber upon the anode element of the circuit due to the electro-negative character of the rubber or like constituent of the latex.

35 The electrolyte selected must be such that, when added to the latex, it is not in itself capable of causing coagulation of the latex except after a considerable interval of time, if at all.

40 Other chemicals or fillers, such for example, as zinc oxide or sulphur, or other vulcanizing agents, with or without accelerators of vulcanization, which do not cause premature coagulation of the latex, may be 45 added before introducing the electrodes, in order that such chemicals or fillers will become incorporated with the deposited rubber.

The cathode element may be made up with or without a depolarizing agent.

50 For example, a weak electrolytic action

might be obtained by immersing conductively connected suitable electrodes in a preserved or alkaline latex without the necessity of adding ammonium chloride or another electrolyte.

55 As an example of one method of carrying out the invention, to ordinary commercial alkaline rubber latex prepared with ammonia and having an alkalinity corresponding ap-

proximately to a semi-normal  $(\frac{N}{2})$  solution

60 of ammonia, is added ammonium chloride solution until the content of ammonium chloride is approximately twenty per cent by weight, thus at the same time reducing the 65 alkalinity of the mixture to approximately that of a  $\frac{N}{6}$  solution of ammonia. The elec-

66 trodes employed consist of a zinc plate as the anode and a porous container enclosing a carbon element, and manganese dioxide for depolarizing purposes, as the cathode. The electrodes are immersed in the mixture of alkaline latex and ammonium chloride solution and the circuit is completed by externally 70 connecting the electrodes, thereby setting up an electro-motive force, effecting deposition 75 of the rubber upon the anode.

The deposition of the rubber or like constituent from the latex can be continued until 80 the desired thickness of rubber or the like has been obtained upon the anode element, which may be shaped to give any desired form to the deposited rubber. The article is then 85 complete in the case of vulcanized latex, and in the case of ordinary commercial latex it can then be vulcanized, if desired, by any known method.

90 It is to be understood that the degree of alkalinity of the mixture of latex and electrolyte will depend upon the nature of the electrolyte.

I do not confine myself to the chemicals, 95 metals or materials herein mentioned or to the proportions or degrees of alkalinity herein stated, these being given only as examples.

## Claims:

1. A process for the electro-deposition of rubber or homologous substances from alkaline latex, which consists in the addition to 100

the latex of an electrolyte which will not in itself readily cause coagulation, but which in conjunction with suitably selected electrodes immersed in the mixture, and directly and conductively connected together externally, will act as a self-excitant, setting up an electro-motive force in the circuit sufficient to effect deposition of the rubber or homologous substances upon the anode element, but insufficient to cause a decomposition which would produce gas bubbles at the anode.

2. A process for the electro-deposition of rubber from an alkaline rubber latex which consists in adding to the latex ammonium chloride solution, and introducing into the mixture zinc and carbon electrodes directly and conductively connected together outside the mixture.

The foregoing specification signed at Edinburgh, Scotland, this twentieth day of April, 1927.

WILLIAM ARTHUR WILLIAMS.

25

30

35

40

45

50

55

60